

Jan. 5, 1971

NARIO YAMAGUCHI ET AL

3,552,959

ELECTROPHOTOGRAPHIC COPYING PAPER

Filed March 18, 1968



INVENTORS  
NARIO YAMAGUCHI  
KAZUO TUBUKO  
BY  
Woodham, Blanchard & Flynn  
ATTORNEYS

**1**

3,552,959

**ELECTROPHOTOGRAPHIC COPYING PAPER**  
Nario Yamaguchi and Kazuo Tubuko, Tokyo, Japan, as-  
signors to Kabushiki Kaisha Ricoh, Tokyo, Japan, a  
corporation of Japan

Filed Mar. 18, 1968, Ser. No. 713,893  
Claims priority, application Japan, Mar. 23, 1967,  
42/17,650

Int. Cl. G03g 5/06

U.S. CL. 96—1.6

6 Claims

**ABSTRACT OF THE DISCLOSURE**

An electrophotographic copying paper comprising a support paper and a photoconductive layer (which is a light-sensitive layer) coated on one surface of said support and containing an organic photoconductive material, wherein said photoconductive layer further contains a metal nitrate, with or without an organic acid.

**BACKGROUND OF THE INVENTION****Field of the invention**

The present invention is concerned with a novel electrophotographic copying paper having a highly increased sensitivity to light and having a photoconductive layer which is formed with an organic photoconductive material, wherein said photoconductive layer further contains a specific assistant sensitizer.

**Description of the prior art**

Some of the conventional electrophotographic copying papers have employed organic photoconductive materials such as poly-N-vinyl carbazole as the photoconductive materials to be contained in the light-sensitive or the photoconductive layer of the copying papers. Most of these known organic photoconductive materials have their spectral sensitivity in the limited range of ultraviolet rays, say, 355 m $\mu$ , more or less. For this reason, there has been made a proposal to expand the light-sensitivity of those electrophotographic copying papers which utilize organic photoconductive materials in the formation of their photoconductive layers through to the range of the visible rays by including, in the photoconductive layers, an assistant sensitizer which includes: metal halides such as zinc chloride, stannous chloride, aluminum chloride, ferric chloride and stannic chloride; acids such as acetic acid, monochloro acetic acid, dichloro acetic acid and trichloro acetic acid or their anhydrides; quinones such as benzoquinone; aldehydes; and ketones. These additives, however, often failed to enhance the light-sensitivity of the photoconductive layers formed. In some cases, these additives even decreased the sensitivity to light of such photoconductive layers, depending on the type of the sensitizing dyestuffs which were included, together with said additives, in the photoconductive layers. Also, in the event that zinc chloride or ferric chloride was included in the photoconductive layer, such a photoconductive layer exhibited a difficulty in the electrostatic charging thereof and required a relatively long period of time till the potential of the layer was saturated. On the other hand, the inclusion of such an additive as dichloro acetic acid or trichloro acetic acid in the photoconductive layers often caused a reduction in the resistance of the photoconductive layers to light-fatigue. Whereas, the inclusion of a metal halide such as ferric chloride or stannic chloride in the photoconductive layer caused an intensive gelation of the solution for use in forming photoconductive layers, making the procedure of applying the solution onto a support such as paper difficult.

**2****SUMMARY OF THE INVENTION**

It is, therefore, the object of the present invention to provide an electrophotographic copying material having a photoconductive layer formed on one surface thereof, 5 said layer containing, in combination with an organic photoconductive material which is the principal component thereof, an assistant sensitiser which consists of a metal nitrate and which is capable of markedly improving the sensitivity to light of said photoconductive layer, without adversely affecting the electrostatic property of this layer, that is to say, without in any way deteriorating the charge characteristics of the photoconductive layer or without reducing the resistance of the photoconductive layer to light-fatigue (in this latter case, the charge characteristic of the photoconductive layer is deteriorated also).

The metal nitrates which can be employed in the present invention are comprised of those metals which are contained in the Group I, Group II, Group III and Group VIII of the periodic table.

The assistant sensitizers which are particularly suitable for the objects of the present invention are those metal nitrates such as magnesium nitrate, zinc nitrate, sodium nitrate, potassium nitrate, cuprous nitrate, ferrous nitrate, ferric nitrate, cobalt nitrate, nickel nitrate, aluminum nitrate and manganese nitrate. The present invention contemplates the complete elimination of the aforesaid drawbacks and inconveniences which have been encountered in the conventional electrophotographic copying papers, 20 by the inclusion—in the photoconductive layer—of such an assistant sensitizer as enumerated above in an amount ranging from 0.1% to 15% by weight of the organic photoconductive material which is contained in the photoconductive layer.

The present invention also contemplates the provision of an electrophotographic copying paper whose photoconductive layer further contains—in addition to the aforesaid metal nitrate—an organic acid such as organic carboxylic acids, organic sulphonic acids, organic phosphoric acids, nitrophenols and acid anhydrides in an amount ranging from 5% to 50% by weight of the metal nitrate which is contained in the photoconductive layer.

The aforesaid organic acid which can be used in the present invention includes:

Organic carboxylic acids, such as acetic acid and the substitution products thereof, monochloro-acetic acid, dichloroacetic acid, trichloroacetic acid, phenylacetic acid, and 6-methylcoumarinylacetic acid (4); maleic acid; cinnamic acid, benzoic acid, 1-(4'-diethylamino-benzoyl)-benzene-2-carboxylic acid, phthalic acid, and tetrachlorophthalic acid,  $\alpha$ , $\beta$ -dibromo- $\beta$ -formyl-acrylic acid (muco-bromic acid), dibromo-maleic acid, 2-bromo-benzoic acid, gallic acid, 3-nitro-2-hydroxy-1-benzoic acid, 2-nitro-phenoxyacetic acid, 2-nitro-benzoic acid, 3-nitrobenzoic acid, 4-nitro-benzoic acid, 3-nitro-4-ethoxy-benzoic acid, 2-chloro-4-nitro-1-benzoic acid, 3-nitro-4-methoxy-benzoic acid, 4-nitro-1-methyl-benzoic acid, 2-chloro-5-nitro-1-benzoic acid, 3-chloro-6-nitro-1-benzoic acid, 4-chloro-3-nitro-1-benzoic acid, 5-chloro-3-nitro-2-hydroxy-benzoic acid, 4-chloro-2-hydroxy-benzoic acid, 2,4-dinitro-1-benzoic acid, 2-bromo-5-nitro-benzoic acid, 4-chlorophenylacetic acid, 2-chloro-cinnamic acid, 2-cyano-cinnamic acid, 2,4-dichlorobenzoic acid, 3,5-dinitro-benzoic acid, 3,5-dinitro-salicylic acid, malonic acid, mucic acid, aceto-salicylic acid, benzilic acid, butane-tetra-carboxylic acid, citric acid, cyano-acetic acid, cyclohexane-dicarboxylic acid, cyclohexane-carboxylic acid, 9,10-dichloro-stearic acid, fumaric acid, itaconic acid, levulinic acid (levulinic acid), malic acid, succinic acid,  $\beta$ -bromo-propionic acid,  $\alpha$ -bromo-stearic acid, citraconic acid, di-bromo-succinic acid, pyrene-2,3,7,8-tetra-carboxylic acid, tartaric acid;

Organic sulphonic acids, such as 4-toluenesulphonic acid, and benzene sulphonic acid, 2,4-dinitro-1-methylbenzene-6-sulphonic acid, 2,6-dinitro-1-hydroxy-benzene-4-sulphonic acid, 2-nitro-1-hydroxy-benzene-4-sulphonic acid, 4-nitro-1-hydroxy-benzene-2-sulphonic acid, 3-nitro-2-methyl-1-hydroxy-benzene - 5 - sulfonic acid, 6-nitro-4-methyl-1-hydroxy-benzene - 2 - sulfonic acid, 4-chloro-1-hydroxy-benzene-3-sulfonic acid, 2-chloro-3-nitro-1-methylbenzene-5-sulfonic acid, 2-chloro - 1 - methylbenzene-4-sulfonic acid;

Organic phosphonic acids, such as 4-chloro-3-nitrobenzene-phosphonic acid;

Nitrophenols, such as 4-nitrophenol, and picric acid;

Acid anhydrides, for example; acetic anhydride, succinic anhydride, maleic anhydride, phthalic anhydride, tetra - chlorophthalic anhydride, and chrysene - 2,3-8-9-tetra-carboxylic anhydride, dibromo maleic acid anhydride.

Description will hereunder be directed to one example of the procedures for preparing the electrophotographic copying papers of the present invention.

An organic photoconductive material is dissolved in a solvent such as monochloro benzene, dimethyl formamide and methylene chloride in such a way that the concentration of the organic photoconductive material in the solvent is in the range of from 5% to 10% by weight of said solvent. To this solution is added a sensitizing dyestuff—in the form of, for example, a methanol solution—in an amount, in terms of the dyestuff, ranging from 0.1% to 2% by weight of the photoconductive material used. Then, a metal nitrate such as those described above is added—in the form of a methanol solution, for example—to the resulting solution in an amount ranging from 0.1% to 15% by weight of said photoconductive material. The addition, if desired to do so, of the aforesaid organic acid is performed at the time when the aforesaid metal nitrate is introduced into the solution. After thoroughly mixing the resulting solution by stirring, the mixed liquid is applied onto one surface of a support—such as a sheet of paper, metal plate, a film made with either a synthetic resin or a naturally occurring resin—which has been already given an electroconducting treatment. The coated support paper is then dried at a temperature ranging from 100° C. to 150° C. for a period of time ranging from 2 to 5 minutes to regulate the moisture content thereof to a level ranging from 4.0% to 4.5% by weight of the support. Thus, an electrophotographic copying paper having a highly increased sensitivity to light is obtained. It is needless to say that this electrophotographic copying paper is conveniently applicable to those high speed electrophotographic copying apparatuses which have been recently developed.

The organic photoconductive materials which can be used in the present invention include poly-N-vinyl carbazole, poly-N-dimethyl-amino-acenaphthylene, poly-N-vinyl-nitro carbazole, polyvinyl naphthalene, polyvinyl-N-dimethyl-amino carbazole, poly-N-diethyl-amino-acenaphthylene, polyvinyl anthracene and polyvinyl nitro-naphthalene. The present invention is featured in that those organic photoconductive materials of both the electron donating type and the electron attracting type can be employed equally. As the sensitizing dyestuffs, substantially all of those basic dyes such as Rhodamine B (C.I. No. 45170), Rhodamine G (C.I. No. 45150) Rhodamine S (C.I. No. 45050), Methyl Violet (C.I. No. 42535), Ethyl Violet (C.I. No. 42600), Crystal Violet (C.I. No. 42555), Methylene Blue FZ (C.I. No. 52015), Methylene Blue BH (C.I. No. 52015), Victoria Blue B (C.I. No. 44045), Brilliant Green GX (C.I. No. 42040), Malachite Green (C.I. No. 42000), Basic Flavine 8G (C.I. No. 75670), Concentrated Auramine G (C.I. No. 41005) and Acridine Orange NS (C.I. No. 46005), are usable. According to the present invention, an equally satisfactory effect can be expected from the inclusion of those sensitizing dyestuffs, irrespective of whether these sensitizing

dyestuffs are included independently or in any desired combination in the photoconductive layers.

While, in the present invention, the presence of a metal nitrate in the photoconductive layer increases greatly the light-sensitivity of the manufactured copying papers as compared with the light-sensitivity of the conventional electrophotographic copying papers, it is to be noted that the inclusion—in combination—of an organic acid and a metal nitrate in the photoconductive layers will further enhance the light-sensitivity of the copying papers produced.

As has been described, the present invention provides an electrophotographic copying paper having a highly increased sensitivity to light, by the inclusion of a metal nitrate in the photoconductive layer which is prepared by the use of an organic photoconductive material. Also, the present invention contemplates a further increasing of the light-sensitivity of the photoconductive layer which is formed with an organic photoconductive material, by the joint inclusion of a metal nitrate and an organic acid such as formic acid or acetic acid in the photoconductive layer.

#### BRIEF DESCRIPTION OF THE DRAWING

The accompanying drawing shows the curve which represents the electrostatic characteristics of the electrophotographic copying paper obtained in the following Example 1. The solid line in the drawing denotes the characteristic curve of the electrophotographic copying paper of the present invention, while the broken line represents that of the control copying paper which is used for the purpose of the comparison of the electrostatic characteristics of these two copying papers. More specifically, these two curves both show the changes in the potential of the photoconductive layers which occurred during the period from the time when the copying papers were "charged on," that is to say, when the photoconductive layers were impressed with an electric charge by corona discharge, with the subsequent "charge off" or the cessation of the charging and then leaving the copying papers in darkness for a while, to the time of the exposure of these copying papers to light.

#### DESCRIPTION OF THE PREFERRED EMBODIMENTS

##### Example 1

5 gr. of poly-N-vinyl carbazole was dissolved in 95 gr. of monochloro benzene. To this solution was added 1.4 gr. of Rhodamine B (1% methanol solution) to serve as the sensitizing dyestuff. To the resulting mixed solution was added further 1.05 gr. of aluminum nitrate (5% methanol solution), and the resulting mixed liquid was stirred thoroughly. This mixed liquid was applied onto one surface of an art paper which had been already given an electroconducting treatment to a thickness of 4 $\mu$ . The coated support paper was then dried at 120° C. for 5 minutes to regulate its moisture content to 4.0%. The electrostatic characteristic of the electrophotographic copying paper thus obtained is shown by the solid line in FIG. 1. The velocity of the light decay of the copying paper obtained in this example was noted to be about 10 times greater than that which was indicated by the electrostatic characteristic (refer to the broken line in the drawing) of the control copying paper whose photoconductive layer which was formed with poly-N-vinyl carbazole contained a sensitizing dyestuff which consisted of Rhodamine B alone.

##### Example 2

5 gr. of poly-N-vinyl carbazole was dissolved in 95 gr. of Methyl Cellosolve. To this solution were added 1.5 gr. (1% methanol solution) of Aizen Magenta, a product of Hodogaya Chemical Co., Ltd. and also 1.0 gr. (1% methanol solution) of Methylene Blue FZ and further 1.05 gr. (5% methanol solution) of zinc nitrate. The mixture was stirred completely. Thus, a mixed liquid was pre-

## 5

pared. This liquid was applied, to a thickness of  $3\mu$ , onto one surface of a mat tracing paper of 60 gr./m.<sup>2</sup> which had been given an electroconducting treatment, and was dried at 100° C. to regulate its moisture content. The copying paper thus obtained showed a light decay which was noted to be about 12 times greater in velocity than that of the control copying paper which was formed without the inclusion of zinc nitrate. The copying paper obtained in this example was found to be satisfactory with respect to the charge characteristic.

## Example 3

5 gr. of poly-N-vinyl-nitro carbazole was dissolved in 95 gr. of dimethyl formamide. To this solution were added 1.0 gr. (1% methanol solution) of Crystal Violet and also 2.0 gr. (5% methanol solution) of magnesium nitrate, and the mixture was stirred thoroughly. Thus, a mixed liquid was prepared. This liquid was applied, to a thickness of  $4\mu$ , onto one surface of an acetate film which had been given an electroconducting treatment, and the coated support was dried to regulate the moisture content thereof. The copying paper obtained in this way showed a light decay which was noted to be about 8 times greater in velocity as compared with that of the control copying paper which contained no magnesium nitrate in the photoconductive layer. The copying paper which was obtained in this example according to the present invention gave a well-contrasted copied image.

## Example 4

5 gr. of polyvinyl carbazole was dissolved in 95 gr. of monochloro benzene. To this solution were added 1.0 gr. (1% methanol solution) of Rhodamine B and also 1.05 gr. (5% methanol solution) of aluminum nitrate and 0.5 gr. (5% methanol solution) of acetic acid. The resulting mixed liquid was stirred at 70° C. for 5 minutes and then was cooled to room temperature. The resulting liquid was applied onto one face of an art paper to a thickness of  $5\mu$ , and was dried at 120° C. for 2 minutes to regulate the moisture content to 4.5%. The copying paper thus obtained showed a light decay which was noted to be about 15 times greater in velocity than that of the control copying paper in which the sensitizing dyestuff contained in this photoconductive layer consisted of Rhodamine B alone. The copying paper also showed only a negligible amount of light-fatigue. The copied image obtained from this copying paper of the instant example was a well-contrasted one.

Aside from the foregoing one, electrophotographic copying papers were prepared from each combination of aluminum nitrate and an acid, i.e. benzene sulphonic acid, 4-chloro-3-nitro-benzene-phosphoric acid, picric acid and dibromo maleic acid anhydride, respectively, which were used in place of the acetic acid contained in the composition of the aforesaid mixed liquid.

It was found that the sensitivity to light of the photoconductive layers of these electrophotographic copying papers was substantially equal to that of the above-described copying paper obtained from the combination of aluminum nitrate and acetic acid.

## What is claimed is:

1. An electrophotographic copying material comprising a support and a photoconductive layer formed on one surface of said support, said layer consisting essentially of an organic photoconductive polymeric material containing therein from 0.1 to 15% by weight, based on the weight of said photoconductive polymeric material, of at least one metal nitrate selected from the group consisting of magnesium nitrate, zinc nitrate, sodium nitrate, potassium nitrate, cuprous nitrate, ferrous nitrate, ferric nitrate, cobalt nitrate, nickel nitrate, aluminum nitrate and manganese nitrate, and from 5 to 50% by weight, based on the weight of said metal nitrate, of at least one organic acid selected from the group consisting of organic carboxylic acids, organic sulphonic acids, organic phosphoric acids, nitrophenols and acid anhydrides.

2. An electrophotographic copying material according to claim 1, wherein said organic photoconductive poly-

## 6

meric material is at least one substance selected from the group consisting of poly-N-vinyl carbazole, poly-N-dimethyl-amino-acenaphthalene, poly-N-vinyl-nitro carbazole, polyvinyl naphthalene, polyvinyl-N-dimethyl-amino carbazole, poly-N-diethyl-amino-acenaphthalene, polyvinyl anthracene and polyvinyl nitronaphthalene.

3. An electrophotographic copying material according to claim 1, wherein said organic photoconductive polymeric material further contains from 0.1 to 2% by weight, based on the weight of said photoconductive polymeric material, of at least one sensitizing dyestuff selected from the group consisting of Rhodamine B (C.I. No. 45170), Rhodamine G (C.I. No. 45150), Rhodamine S (C.I. No. 45050), Methyl Violet (C.I. No.

10 42535), Ethyl Violet (C.I. No. 42600), Crystal Violet (C.I. No. 42555), Methylene Blue FZ (C.I. No. 52015), Methylene Blue BH (C.I. No. 52015), Victoria Blue B (C.I. No. 44045), Brilliant Green CX (C.I. No. 42040), Malachite Green (C.I. No. 42000), Basic Flavine 8G (C.I. No. 75670), Concentrated Auramine G (C.I. No. 41005), and Acridine Orange NS (C.I. No. 46005).

4. An electrophotographic copying material comprising support and a photoconductive layer formed on one surface of said support, said layer consisting essentially of an organic photoconductive polymeric material containing therein from 0.1 to 15% by weight, based on the weight of said photoconductive polymeric material, of at least one metal nitrate selected from the group consisting of magnesium nitrate, zinc nitrate, sodium nitrate, potassium nitrate, cuprous nitrate, ferrous nitrate, ferric nitrate, cobalt nitrate, nickel nitrate, aluminum nitrate and manganese nitrate, and from 5 to 50% by weight, based on the weight of said metal nitrate, of at least one organic acid selected from the group consisting of organic carboxylic acids, organic sulphonic acids, organic phosphoric acids, nitrophenols and acid anhydrides.

5. An electrophotographic copying material according to claim 4, wherein said organic photoconductive polymeric material is at least one substance selected from the group consisting of poly-N-vinyl carbazole, poly-N-dimethyl-amino-acenaphthalene, poly-N-vinyl-nitro carbazole, polyvinyl naphthalene, polyvinyl-N-dimethyl-amino carbazole, poly-N-diethyl-amino-acenaphthalene, polyvinyl anthracene and polyvinyl nitronaphthalene.

6. An electrophotographic copying material according to claim 4, wherein said organic photoconductive polymeric material further contains from 0.1 to 2% by weight, based on the weight of said photoconductive polymeric material, of at least one sensitizing dyestuff selected from the group consisting of Rhodamine B (C.I. No. 45170), Rhodamine G (C.I. No. 45150), Rhodamine S (C.I. No. 45050), Methyl Violet (C.I. No. 42535), Ethyl Violet (C.I. No. 42600), Crystal Violet (C.I. No. 42555), Methylene Blue FZ (C.I. No. 52015), Methylene Blue BH (C.I. No. 52015), Victoria Blue (C.I. No. 44045), Brilliant Green GX (C.I. No. 42040), Malachite Green (C.I. No. 42000), Basic Flavine 8G (C.I. No. 75670), Concentrated Auramine G (C.I. No. 41005), and Acridine Orange NS (C.I. No. 46005).

## References Cited

## UNITED STATES PATENTS

|           |         |                |        |
|-----------|---------|----------------|--------|
| 2,776,251 | 1/1957  | Schwartz       | 204—2  |
| 3,152,903 | 10/1964 | Shepard et al. | 96—64  |
| 3,169,060 | 2/1965  | Hoegl          | 96—1.6 |
| 3,287,121 | 11/1966 | Hoegl          | 96—1.5 |

GEORGE F. LESMES, Primary Examiner

70 C. E. VAN HORN, Assistant Examiner

U.S. CL. X.R.

96—1.5; 252—501